

## UNITED STATES PATENT OFFICE.

NIKOLAI WOROSHTZOW, OF BERLIN, GERMANY.

## PROCESS FOR COLORING ORGANIC FIBERS OR ARTICLES SUCH AS SKINS, FURS, PAPER, ETC., CONSISTING OF ANIMAL AND VEGETABLE FIBERS.

No Drawing.

Application filed June 30, 1925. Serial No. 40,686.

This invention relates to processes for coloring organic fibers whether woven, loose or manufactured products or articles such as skins, furs, paper etc. consisting of animal 5 and vegetable fibers.

Aromatic nitro-compounds have hitherto only been used very little for the coloring of fibers of all kinds. Such compounds have hitherto been chiefly used for producing a few 10 yellow dyes, dinitro or polynitro derivates of certain phenols and amines having been chiefly employed for this purpose.

I have discovered that certain nitro-compounds of the naphthalene series and particularly such as contain in their compounds, 15 in addition to the nitro-group, one or more sulfonic acid-groups, and which in themselves do not possess any dyeing properties, are capable of producing pleasing tints, ranging 20 from brown to dark brown on fiber articles, if the article to be colored or dyed such as paper, fur or the like, is impregnated with the nitro-compound in question and is exposed to sunlight after drying. The parts of 25 the material or article prepared in the aforesaid manner which are exposed to the light assume after a short time pleasing dark tints. The beauty of the tints can be increased and the time of exposure to the light can be simultaneously shortened if, instead of treating 30 the fibrous materials with nitro-compounds only, a mixture of nitro-compounds with aromatic amines is used. The amines may be employed in a free condition or in the form 35 of a salt. Particularly suitable forms have been found to be aniline, its homologues and substitution derivatives, phenylenediamines, monoamines and diamines of the naphthalene series etc. When these amines are added tints 40 ranging from dark to black are obtained.

As the initial substances used for treating the fibers can be removed only from the parts that have not been exposed, while the dyeing agent adheres firmly to the parts that have 45 been exposed to the light, the novel process enables photographic pictures to be produced without the aid of metal salts. The dyestuff formed does not fade at all when exposed to light so that the pictures do not change when 50 they are exposed to light after they have been washed.

As the fibrous articles are treated with solutions of the nitro-compounds and are exposed to light at ordinary temperatures the processes 55 can be advantageously employed for

dyeing furs, skins and the like, as these latter will not be injured by being immersed in hot baths.

In carrying out my novel process I prefer to use such mono-nitro-naphthalene-sulfonic acids as contain the nitro and sulfonic acid group in different six-ring cores. The most favourable position is the grouping in which nitro- and sulfonic acid-groups are in the  $\alpha$ -position relatively to each other. The meta- 65 position, however, is very unfavourable.

*Example 1.*

Wool is impregnated at an ordinary temperature with a three per cent solution of 70 1-nitronaphthalene-7-sulfonic acid, then treated in the absence of actinic rays, and afterwards exposed to sunlight. After an exposure of one quarter to a full hour, according to the intensity of the light, a dark brown 75 color is obtained which is perfectly fast or unchangeable. If instead of nitronaphthalene-sulfonic acid a solution containing, in 100 parts, three parts of 1-nitronaphthalene-7-sulfonic acid and 0.5 parts aniline hydrochlorid is employed the effect of the light is completed in a shorter time and a black tint is obtained. 1-nitronaphthalene-6-sulfonic acid, 1-nitronaphthalene-8-sulfonic acid, 1,6-dinitro-naphthalene-4,8-disulfonic acid and 85 other nitro- and dinitro-naphthalene-sulfonic acids behave similarly.

*Example 2.*

A white skin is treated with a five per cent 90 solution of 1,6-dinitro-naphthalene-4,8-disulfonic acid with the aid of a brush or by immersion and then exposed after drying to sunlight. A brown color is thus obtained which can be darkened by chroming.

If the skin is treated, after impregnation with dinitro-naphthalene-disulfonic acid and drying, with a substantially 0.1 percent solution of paraphenylenediamine-hydrochloride, a black color is obtained after a short exposure to light. If, instead of the entire skin, only parts of it are treated with the diamine solution a skin is obtained which, after its exposure to light, has a black pattern on a dark brown base.

If a screen with transparent patterns, figures or the like, is placed on the impregnated skin and the light beams are thus prevented from striking certain parts of the skin, an article is obtained which is only colored at 110

the transparent parts of the screen when the substances on the skin that have not been chemically changed by the action of light are washed away with water or a weak solution of 5 sodium hydrate or sodium carbonate.

5. The 1,6-dinitro-4,8-disulfonic acid can be replaced by other dinaphthalene- or mono-naphthalene-sulfonic acids. Similarly the 10 paraphenylendiamine can be replaced by 10 other aromatic diamines or monoamines.

*Example 3.*

A sheet of paper that has been prepared by 15 coating it with gelatine is treated with a 3 to 5 per cent solution of 1-nitro-naphthalene- 20 8-sulfonic acid, this solution being applied in any suitable manner as by a brush. After 25 drying the paper is exposed to sunlight through a photographic negative. In this manner a photographic picture is obtained 30 which is fixed by washing the paper with water or a weak solution of sodium hydrate or sodium carbonate. Darker or black tones are obtained by preparing the paper with 35 25 nitro-naphthalene-sulfonic acid and at the same time with aniline hydrochloride or paraphenylendiamine hydrochloride or the like. By this means the effect of the light is also accelerated. An acceleration is also obtained 40 if the addition of amine is replaced by some metal salts such as cupric or cuprous sulfate, ammonium-vanadate or the like that act as a catalytic agent.

Instead of preparing the paper with a 45 coating of gelatine a film of agar-agar, albumin, or other substances may be used. The nitro-sulfonic acid mentioned in this example of the process and the amine can be replaced by other analogous compounds.

40. I claim:

1. Process of the kind described consisting 45 in treating organic fibers with nitro-naphthalene compounds which contain a nitro-group and a sulfonic acid-group, and in exposing the fibers thus treated to light.

2. Process of the kind described consisting

in treating organic fibers with nitro-naphthalene compounds which contain a plurality of nitro-groups and a sulfonic acid-group, and in exposing the fibers thus treated to 50 light.

3. Process of the kind described consisting in treating organic fibers with nitro-naphthalene compounds which contain a plurality of nitro-groups and of sulfonic acid-groups, 55 and in exposing the fibers thus treated to light.

4. Process of the kind described consisting in treating organic fibers with nitro-naphthalene compounds which contain a nitro- 60 group and a sulfonic acid-group, also treating the fibers with an aromatic amine, and exposing the fibers thus treated to light.

5. Process of the kind described consisting in treating organic fiber articles with nitro- 65 naphthaline compounds that contain a nitro-group and a sulfonic acid-group, also treating the fibers with an aromatic amine, producing a pattern on the article by exposing it to light that passes through transparent parts 70 of a screen, and fixing the pattern after exposure of the article to light by washing the article.

6. Process of the kind described consisting in treating paper coated with nitro-naphthalene compounds that contain a nitro-group and a sulfonic acid-group, and in exposing the treated paper to light through a photographic negative and washing said 75 treated paper.

7. Process of the kind described consisting in treating paper coated with a nitro-naphthalene compound containing a nitro-group, a sulfonic acid-group and a catalytic agent, exposing the paper thus treated to light 80 through a photographic negative, and fixing the pattern thus produced by actinic rays on the paper by washing the same.

In testimony whereof I have affixed my signature.

NIKOLAI WOROSHTZOW.